

# UNITED STATES PATENT OFFICE.

ALFRED WILM, OF SCHLACHTENSEE-BERLIN, GERMANY.

## METHOD OF MAKING ALUMINUM-ALLOY ARTICLES.

1,261,987.

Specification of Letters Patent. Patented Apr. 9, 1918.

No Drawing. Application filed May 24, 1912, Serial No. 699,553. Renewed August 23, 1917. Serial No. 187,887.

To all whom it may concern:

Be it known that I, ALFRED WILM, a subject of the King of Prussia, Emperor of Germany, residing in Schlachtensee-Berlin, Germany, have invented certain new and useful Improvements in Methods of Making Aluminum-Alloy Articles; and I do hereby declare the following to be a full, clear, and exact description of the invention, such as will enable others skilled in the art to which it appertains to make and use the same.

The present invention relates to aluminum-alloy articles, and to a method of making the same which is directed to obtaining a uniform close-grained texture of the metal of the articles, of such a character as to impart thereto increased strength, rigidity, and inertness to electrolysis. The departure from the known procedure which characterizes this invention lies in bringing about a close-grained texture of the metal of aluminum-alloy articles with a uniform distribution of the metallic constituents through the mass, by selecting such metals and in such proportional quantities as will admit of the formation of an article from a molten admixture thereof, which will subsequently become intimately and uniformly associated throughout the mass of the article under the influence of a degree of heat less than would be required to destroy the form of the article, and which will ultimately be fixed in such intimate and uniform association in the mass by the withdrawal of heat at a rate which will not allow time for their less intimate or less uniform redistribution therein.

The correlation of the admixture of chosen metals with the particular treatment to which it is subjected can be varied to some extent to effect differing degrees of hardness, ductility and strength in the metal of the article produced, but the limits of permissible variation in the quantities of the metals used to effect advantageous results are well defined, as will appear from the following description.

In order to produce an aluminum-alloy article having the desirable characteristics enumerated above, it has been necessary to discover what metals and what proportions of said metals, when admixed with a major quantity of aluminum, would assume an intimate association and uniform distribution in a mass at some temperature below the congealing point of the mass. Thus I have found that when approximately one-half of

one per cent. of magnesium is added to a molten admixture of aluminum with approximately from 3 to 6 per cent. of copper and a quantity of manganese approximating one-seventh of the copper content, an article formed from said admixture can be given the required texture, resulting in a marked increase in strength and rigidity and resistivity to electrolytic decomposition, by cooling it from a temperature of substantially 500° C. with sufficient rapidity to insure the fixation of the constituents in the uniformly distributed and intimate structural condition present at that temperature.

The several variations of this alloy are prepared commercially from a rich alloy which may be produced in the following manner:

Say seven kilograms of copper are heated in a graphite crucible with one kilogram of manganese, free from carbon, to a light-red heat, at which the copper is completely melted but the manganese only partially so. Into this charge, weighing eight kilograms, four kilograms of aluminum are charged. When the aluminum is melted and the crucible charge is at a red heat it is stirred for a short time with an iron rod, whereupon the temperature of the charge will rise to white heat owing to the heat generated by the reduction of the metallic oxides of copper and manganese by the aluminum. The aluminum oxid thus formed rises readily to the surface of the charge and may be removed as a scum by a rod. Another quantity of four kilograms of aluminum is now added, stirred up and the molten admixture thereupon quickly poured out into a shallow iron mold to chill. This rich alloy contains a relatively large quantity of manganese which would settle out if the charge were allowed to cool slowly.

The rich alloy is melted with an added amount of aluminum to bring the copper content to from 3 to 6 per cent. of the mass, as the requirements of the product may call for. Approximately one-half of one per cent. of metallic magnesium is now added to the molten mass, preferably after it has been removed from the smelting furnace, and the charge is formed into the article, congealing in the form required for the article which may be an ingot, a bar, or a cast shape of any other kind.

As it is usually difficult to cool a cast piece in the mold to a predetermined temperature

throughout, I prefer to reheat the piece throughout, when it is desired to effect the uniform distribution of the metals, to a temperature lying between 420° C. and 560° C. and preferably closely approximating 500° C. and thereafter cool it to the normal temperature with sufficient rapidity to prevent substantial separation of the metallic constituents from the uniformly distributed condition to which they have been brought by the heat treatment, as, for example, by quenching it in water.

The presence of copper in the alloy in excess of six per cent. will generally prevent the obtaining of a fine-grained uniformly-distributed texture, by the application of any temperature below the congealing point, while the addition of magnesium in quantities above two per cent. or much below .5 per cent. will prevent the attainment of the requisite hardness.

While I prefer to add magnesium in the proportion of approximately one-two-hundredth part of the aluminum content of each particular alloy, the difference is so trifling that for commercial practice I add .5 per cent. of the entire mass for any alloy within the limits herein given.

Heretofore, articles made of aluminum-alloys containing a large percentage of aluminum have not possessed uniform distribution of the constituent metals through the mass, and have consequently suffered from electrolytic decomposition when exposed to air and moisture and were of little or no value as fittings exposed to salt water as in marine construction.

The treated alloys herein described resist the action of salt water to a remarkable degree.

Among other metals which may be used in the aluminum alloys herein described and permit uniformity of distribution with the aluminum, are silver, vanadium, nickel, chromium, tungsten, molybdenum and titanium, any of which will produce advantageous characteristics as to strength and rigidity in the treated alloy-article.

Alloys having certain peculiar advantages for commercial purposes may, for example, be compounded as follows:

With alloys of very great hardness which are obtained by the use of an increased proportion of copper and magnesium, that is to say, with copper up to 5% and magnesium up to 2%, an addition of nickel in suitable proportions will serve to reduce the brittleness of the product without interfering with the uniform distribution of the constituents. Thus an alloy of about 93.25 aluminum, 6% copper, 5% magnesium and .25% nickel has the characteristic qualities above referred to, with increased ductility. Or a particularly good alloy is formed by alloying and treating as above described

94.5 parts aluminum, 4 parts copper, .5 magnesium and 1 part nickel.

By employing chromium in about the proportions 94.5 parts aluminum, 4 parts copper, .5 parts magnesium and 1 part 70 chromium, the capacity to take and retain a polish is increased.

For friction surfaces it is of advantage to use titanium in about the proportions 94.5 parts aluminum, 4 parts copper, .5 parts 75 magnesium and 1 part titanium.

In using an alloy containing iron, I have found the following composition particularly suitable for practising my invention, viz.: aluminum 94.25 parts, copper 4 parts, 80 magnesium .25 and iron 1.5 parts.

In fact a material of great value for certain well-defined purposes may be produced by adding magnesium alone to the aluminum in about the proportion of 200 parts of 85 aluminum to 1 part of magnesium and then subjecting the material to the heat treatment above described. The result is to increase the tensile strength and particularly to make the material easier to work or shape. 90 For purposes such as the manufacture of cooking utensils and the like, where ease of working is more important than tensile strength the magnesium is added in less amount, as for example, about .2% to .3%. 95

It is to be understood that where the material is to undergo machining operations, such as rolling, drawing, turning, swaging and the like, the heat treatment should follow such operations, though slight changes 100 in shape, such as flanging or bending, are permissible immediately after the heat treatment.

Having thus described my invention, what I claim is:

105

1. The method of manufacturing articles of aluminum alloys which comprises forming the article from an admixture of aluminum and one or more other metals in quantities which will assume an adequately uniform proportional distribution throughout the mass within a range of temperature lying below the fusing point of the alloy, maintaining the formed article at a temperature within said range until said uniform proportional distribution of the metals is attained, and cooling the article at a rate which will insure fixation of the uniformly distributed proportions; substantially as described.

110

2. The method of manufacturing articles of aluminum-copper alloys which comprises forming the articles from an admixture containing aluminum and copper, the proportions of the constituents of said admixture 115 being compatible with the assumption by said constituents of an adequately uniform proportional distribution through the mass within a range of temperature lying below the congealing point of the mass, main- 120

130

taining the formed article at a temperature within said range until said uniform proportional distribution of the constituents of the admixture is attained, and cooling the article at a rate which will insure fixation of the uniformly distributed alloy; substantially as described.

3. The method of manufacturing articles of aluminum alloys which comprises the making of a molten admixture of suitable proportions of aluminum and one or more other metals, adding to said molten admixture a quantity of magnesium approximately equal to one-two-hundredth part of the aluminum content of said admixture, subjecting an article formed from said admixture to a temperature somewhat below the congealing point of said admixture until an adequately uniform proportional distribution of the metals is attained throughout the mass and cooling the article to the normal temperature at a rate which will insure fixation of the uniformly distributed proportions; substantially as described.
4. The method of manufacturing articles of aluminum alloys which comprises the making of a molten admixture of suitable proportions of aluminum, copper and manganese, the quantity of manganese being approximately equal to one-seventh of the copper content of the admixture, adding to said admixture a quantity of magnesium approximately equal to one-two-hundredth part of the aluminum content of the admixture, sub-

jecting an article formed from said admixture to a temperature somewhat below the congealing point of said admixture until an adequately uniform proportional distribution of the metals is attained throughout the mass and cooling the article to the normal temperature at a rate which will insure fixation of the uniformly distributed proportions; substantially as, described.

5. The method of manufacturing articles of aluminum alloys which comprises the making of a molten admixture of aluminum, copper and manganese, the copper content of which is limited to from 3 to 6 per cent. and the manganese content being proportional to the amount of copper in the ratio of one part manganese to seven parts copper adding to said admixture approximately .5 per cent. of magnesium, subjecting an article formed from said admixture to a temperature lying above 420° C. until an adequate uniform proportional distribution of the metals is attained throughout the mass and cooling the article at a rate which will insure fixation of the uniformly distributed proportions; substantially as described.

In testimony whereof I affix my signature, in presence of two witnesses.

ALFRED WILM.

Witnesses:

HENRY HASPER,  
WOLDEMAR HAUPT.

It is hereby certified that in Letters Patent No. 1,261,987, granted April 9, 1918, upon the application of Alfred Wilm, of Schlachtensee-Berlin, Germany, for an improvement in "Methods of Making Aluminum-Alloy Articles," an error appears in the printed specification requiring correction as follows: Page 2, line 61, for the numeral and character "5%" read .5%; and that the said Letters Patent should be read with this correction therein that the same may conform to the record of the case in the Patent Office.

Signed and sealed this 30th day of April, A. D., 1918.

[SEAL.]

F. W. H. CLAY,

*Acting Commissioner of Patents.*

Cl. 75—1.